

## 1

3,039,961

NON-CORROSIVE LUBRICATING COMPOSITIONS  
 Robert J. Harker, Terre Haute, Ind., assignor to Commercial Solvents Corporation, New York, N.Y., a corporation of Maryland  
 No Drawing. Filed May 8, 1959, Ser. No. 811,802  
 5 Claims. (Cl. 252—47.5)

My invention relates to non-corrosive lubricating compositions. More particularly, it relates to non-corrosive lubricating compositions comprising a mercapto oxazoline having the following structural formula



where  $\text{R}_1$  is a member selected from the group consisting of  $\text{CH}_3$ ,  $\text{CH}_2\text{OH}$ , and  $\text{C}_2\text{H}_5$ , and  $\text{R}_2$  is a member selected from the group consisting of  $\text{CH}_2\text{OH}$ ,  $\text{CH}_3$ , and  $\text{H}$ .

It is well known to the art that substantially all hydrocarbon lubricating oils are susceptible to harmful oxidation. The degree of susceptibility depends on the process used for refinement and the degree to which readily oxidizable substances are removed. A satisfactory refined lubricating oil can be obtained by refining a crude hydrocarbon oil in the presence of sulfuric acid and treating the refined oil with various compositions; among them silica gel, natural clay, activated charcoal and  $\text{AlCl}_3$ . Such a lubricating oil, however, tends to form acidic substances when subjected to oxidizing conditions. These acidic substances are undesirable and have a corrosive effect upon the metals with which the lubricating oil comes in contact during lubrication. This factor not only shortens the useful life of the lubricating composition, but causes the deterioration of much expensive machinery.

Generally, a suitable non-corrosive lubricating composition minimizes the corrosive effect of oxidation products upon the metals with which a lubricant comes in contact during lubrication and forms a continuous film upon metal surfaces which will resist breakage over extended periods of time even though continuously exposed to the oxidation products normally formed in a lubricating oil.

I have now discovered that a highly satisfactory non-corrosive lubricant which will form a protective film on metal surfaces, said film being resistant to breakage by oxidation products over an extended period of time, can be prepared by adding a mercapto oxazoline having the following structural formula



where  $\text{R}_1$  is a member selected from the group consisting of  $\text{CH}_3$ ,  $\text{CH}_2\text{OH}$ , and  $\text{C}_2\text{H}_5$ , and  $\text{R}_2$  is a member selected from the group consisting of  $\text{CH}_3$ ,  $\text{CH}_2\text{OH}$ , and  $\text{H}$ , to a lubricating oil. Examples of the above-described mercapto oxazolines which are operative in my invention are 2-mercaptop-4-hydroxymethyl-4-methyl-2-oxazoline, 2-mercaptop-4,4-dimethyl-2-oxazoline, 2-mercaptop-4,4-dihydroxymethyl-2-oxazoline, 2-mercaptop-

## 2

ethyl-2-oxazoline, 2-mercaptop-4-ethyl-4-hydroxymethyl-2-oxazoline, etc.

In accordance with my invention, the mercapto oxazolines can be added to the desired lubricant in amounts of from about 0.2 to 10% by weight of the lubricating oil. However, I prefer to use from about 0.5 to 2% by weight of the mercapto oxazolines.

The corrosiveness of the lubricant can be tested by means of various devices. One of these devices is the Underwood oxidation test apparatus.

The Underwood oxidation test apparatus comprises essentially an oil sump containing an electric heater, a gear pump driven by a  $\frac{1}{3}$  horsepower electric motor, a tube containing four orifices, a connecting means connecting the oil sump and the tube, a 30 mesh wire screen positioned between the orifices and the oil sump, and a rectangular box containing all of the aforementioned, except the connecting means and the gear pump. The apparatus is fitted with several control attachments, such as an adjustable thermostatic control attached to a thermocouple for maintaining the desired temperature of the oil, a pressure gauge, a by-pass valve for adjustment to the desired pressure and a control switch for the electric immersion heaters.

The Underwood oxidation test is conducted by charging the desired amount of the test oil containing a suitable oxidation accelerator into the apparatus, placing two copper-lead bearings backed with a copper strip in position opposite the orifices, starting the pump and regulating the temperature and pressure. The test can be conducted for any prescribed length of time after which the bearings are cleaned and weighed. By calculating the loss in weight of the bearings the amount of corrosion produced by a lubricating composition containing an oxidation accelerator can be compared to the amount of corrosion produced by a lubricating composition tested under the same conditions containing an oxidation inhibitor.

The oil base which can be used to prepare the non-corrosive lubricating composition of my invention is preferably a hydrocarbon lubricating oil which will not readily decompose over extended periods of time. The hydrocarbon oil used in preparing the non-corrosive lubricants of my invention can also contain constituents to improve the pour point, etc. Materials used in the art for these purposes which are compatible with the hydrocarbon oil will be found to be useful in the non-corrosive lubricant of my invention.

The following examples are set out to illustrate my invention. It is not intended that the invention be limited to the materials, procedures and proportions set out therein. Various equivalents of my invention will obviously occur to those skilled in the art and I intend to include such equivalents within the scope of my invention.

## Example 1

2,500 mls. of test lubricant containing Kendall SAE No. 10 oil and 0.01% by weight  $\text{Fe}_2\text{O}_3$  as iron naphthenate was charged to the Underwood oxidation apparatus. Two previously weighed copper-lead bearing balls were fixed in position opposite the orifices. The heaters were turned to a temperature of  $325^\circ \text{ F}$ . and the pressure was regulated to 10 p.s.i. The test was continued for 10 hours, after which the balls were cleaned by a special solvent consisting of equal parts of denatured alcohol, toluene and ethyl acetate and weighed to determine the weight loss due to corrosion. The table below shows the results of the test and shows the amount of corrosion

produced by the lubricating composition containing an lubricating oil of a mercapto oxazoline having the following general formula



|                          | Test 1  | Test 2  |
|--------------------------|---------|---------|
| Weight before test/gms.  | 41.9021 | 41.9520 |
| Weight after test/gms.   | 41.7585 | 41.8063 |
| Weight loss.....         | 0.1436  | 0.1457  |
| Percent weight loss..... | 0.342   | 0.347   |

*Example II*

2,500 mls. of test lubricant containing Kendall SAE No. 10 oil, 0.01%  $\text{Fe}_2\text{O}_3$  as iron naphthenate by weight and 1% by weight 2-mercaptop-4-hydroxymethyl-4-methyl-2-oxazoline was charged to the Underwood apparatus. The Underwood oxidation test was performed as described in Example I. The table below shows the results of the test and shows the amount of corrosion produced by a lubricating composition containing an oxidation accelerator and a corrosion inhibitor.

|                          | Test 1  | Test 2  |
|--------------------------|---------|---------|
| Weight before test/gms.  | 41.8919 | 42.6444 |
| Weight after test/gms.   | 41.8907 | 42.6433 |
| Weight loss.....         | 0.0012  | 0.0011  |
| Percent weight loss..... | 0.003   | 0.003   |

Now having described my invention, what I claim is:

1. A lubricating composition consisting essentially of a hydrocarbon lubricating oil and from about 0.2% to 10% by weight on the weight of the hydrocarbon lubri-

10 where  $\text{R}_1$  is a member selected from the group consisting of  $\text{CH}_3$ ,  $\text{CH}_2\text{OH}$  and  $\text{C}_2\text{H}_5$ , and  $\text{R}_2$  is a member selected from the group consisting of  $\text{CH}_3$ ,  $\text{CH}_2\text{OH}$  and  $\text{H}$ .

2. The lubricating composition of claim 1 wherein the mercapto oxazoline is present in amounts of from about 0.5% to about 2% by weight.

3. The lubricating composition of claim 1 wherein the mercapto oxazoline is 2-mercaptop-4-hydroxyl-4-methyl-2-oxazoline.

4. The lubricating composition of claim 1 wherein the mercapto oxazoline is 2-mercaptop-4,4-dimethyl-2-oxazoline.

5. The lubricating composition of claim 1 wherein the mercapto oxazoline is 2-mercaptop-4,4-dihydroxymethyl-2-oxazoline.

References Cited in the file of this patent

UNITED STATES PATENTS

|           |                 |                |
|-----------|-----------------|----------------|
| 2,206,152 | Bennett         | July 2, 1940   |
| 2,348,917 | Mathes          | May 16, 1944   |
| 2,364,399 | Williams et al. | Dec. 5, 1944   |
| 2,776,977 | D'Amico         | Jan. 8, 1957   |
| 2,860,962 | Bluestone       | Nov. 18, 1958  |
| 2,953,573 | Bluestone       | Sept. 20, 1960 |